

1

2,759,031

## PREPARATION OF HIGHLY BRANCHED ALIPHATIC HYDROCARBONS

George J. Benoit, Jr., San Anselmo, Calif., assignor to California Research Corporation, San Francisco, Calif., a corporation of Delaware

No Drawing. Application December 30, 1954,  
Serial No. 478,889

6 Claims. (Cl. 260—676)

This invention relates to a process for preparing highly branched aliphatic hydrocarbons from lower paraffins which comprises heating a lower paraffin or mixture of lower paraffins in the presence of a lower dialkyl peroxide, alkyl hydroperoxide or diacyl peroxide. In particular, this invention relates to a process for preparing highly branched aliphatic hydrocarbons which comprises heating a lower paraffin or mixture of lower paraffins and propane in the presence of a lower dialkyl peroxide.

Highly branched aliphatic hydrocarbons are used extensively in the production of hydrocarbon motor fuels. It is well known that the "knocking" characteristics of hydrocarbon motor fuels represent a dissipation of considerable energy, and in view of the modern trend toward more efficient, higher compression engines, it becomes extremely important to minimize such knocking. It has been found that this dissipation of energy is most serious in the case of straight-chain aliphatic hydrocarbons and becomes progressively less severe with branched or unsaturated hydrocarbons, cyclic paraffins and aromatic hydrocarbons. Inasmuch as straight-chain aliphatic hydrocarbons make up the bulk of hydrocarbons available for use as motor fuels, it is customary to blend them with those hydrocarbons having superior antiknock characteristics (or, in different terminology, higher octane numbers) in order to provide a satisfactory product. The branched aliphatic hydrocarbons are especially valuable for this purpose since not only do they have a high octane value, but also they are compatible with tetraethyl lead which is also added to produce high octane fuels. However, since the amount of high octane blending stocks is relatively limited, it would be desirable if a method were available for converting the less attractive, essentially straight-chain materials to those of a branched character, and it is, therefore, an object of this invention to provide such a method.

The present invention is based on the discovery that the foregoing object can be achieved, with highly branched aliphatic hydrocarbons being produced from lower paraffinic hydrocarbons, by a process wherein a lower paraffin or a mixture of such paraffins is heated in the presence of a peroxide to a temperature affording decomposition of the peroxide at a reasonable rate, said temperatures normally being in the range of from about 150—400° F. depending on the particular peroxide employed. The reaction can be conducted at either atmospheric or superatmospheric conditions, and is preferably effected by continuously agitating the reaction mixture for a period of from about 2 to 60 hours. The relative amount of peroxide initiator to hydrocarbon reactant employed can be varied from about 0.02 to 0.5 mole of peroxide for each mole of the paraffinic reactant, though the reaction of the present invention will go forward in limited degree even outside these limits. A preferred range is from about 0.05 to 0.2 mole of the peroxide per mole of the lower paraffin or paraffins.

As the hydrocarbon reactant there can be employed any one or more of the lower paraffin compounds con-

2

taining from about 3 to 5 carbon atoms per molecule, not more than one of which carbon atoms is in a branched position. Representative reactants of this character include propane, n-butane, isobutane, n-pentane and 5 2-methyl butane. Particularly good results have been obtained when propane is employed either alone or in admixture with isobutane.

As the peroxide material, there can be employed a dialkyl peroxide, an alkyl hydroperoxide, a diacyl peroxide, or mixture of such peroxides. Preferably, however, the peroxide employed is one of the dialkyl variety such, for example, as di-(tert.-butyl) peroxide, methyl ethyl peroxide, di-(sec.-butyl) peroxide, or the like, though di-(tert.-butyl) peroxide is preferred since it has the 15 advantage of commercial availability and is also relatively stable. It has been observed that the highest conversions are obtained with the use of a dialkyl peroxide, with somewhat lower conversions being obtained with alkyl hydroperoxides (e. g., tert.-butyl hydroperoxide), and 20 with still smaller conversions being obtained with acyl peroxides (e. g., benzoyl peroxide and lauroyl peroxide).

As regards the nature of the product produced by a practice of the present invention, the term "highly branched aliphatic hydrocarbon" is employed herein and in the appended claims to describe said products, said term indicating paraffinic hydrocarbons which contain at least 5 and preferably 6 or more carbon atoms in the molecule, with at least 2 of said carbon atoms being in a branched position.

30 The invention is illustrated in various of its embodiments by the following examples.

## Example I

100 grams of di-(tert.-butyl) peroxide were placed in 35 a stainless steel bomb equipped with a heater and means of agitation. The bomb was repeatedly flushed with nitrogen to replace air. Isobutane (300 grams) and propane (300 grams) were then pumped into the bomb. The bomb was heated to 300° F. at a pressure of 1100 40 p. s. i. g. and held at that temperature for 12 hours, following which it was cooled to room temperature. Gas was bled off into a gas holder; a total of 237 liters at 55° F. was collected. The gas was found to be largely isobutane and propane with smaller amounts of hydrogen, 45 methane, ethane, ethylene, propene, butene and C<sub>6</sub> hydrocarbons also present. Of the propane charged, 73% was recovered; 90% of the isobutane charged was recovered.

The bomb liquid product amounted to 146 grams. It was water-washed repeatedly. The oil phase from the 50 washing was dried over K<sub>2</sub>CO<sub>3</sub>. The dried material (33 grams) was distilled through an 18-inch zigzag column, using a 9:1 reflux ratio. 16 grams of highly branched hydrocarbons were obtained within the boiling point range, 154—223° F. (C<sub>6</sub> to C<sub>8</sub>). Of this amount, six 55 grams were triptane (2,2,3-trimethylbutane).

## Example II

Following the procedure of Example I, from 300 parts 60 by weight of isobutane, 300 parts by weight of propane and 100 parts by weight of di-(tert.-butyl) peroxide heated at a temperature of 266° F. and a pressure of about 900 p. s. i. for 54 hours were produced 9 grams of highly branched C<sub>6</sub> to C<sub>8</sub> paraffins, including 6 grams of triptane.

## Example III

Following the procedure of Example I, from 300 parts 65 by weight of isobutane, 300 parts by weight of propane and 100 parts by weight of di-(tert.-butyl) peroxide heated at a temperature of 347° F. and a pressure of 1400 p. s. i. g. for 12 hours were produced 13.9 grams

of highly branched C<sub>6</sub> to C<sub>8</sub> paraffins, including 6.1 grams of triptane.

*Example IV*

Following the procedure of Example III, substituting an equimolar amount of di-(tert.-amyl) peroxide for di-(tert.-butyl) peroxide, essentially the same amount of branched paraffins was obtained.

*Example V*

Following the procedure of Example I, from 600 parts by weight of propane and 100 parts by weight of di-(tert.-butyl) peroxide heated at a temperature of 305° F. and a pressure of 1500 p. s. i. g. for 12 hours were produced 14.1 grams of C<sub>6</sub> to C<sub>8</sub> highly branched paraffins containing 12.5 grams of C<sub>6</sub> paraffins, largely 2,3-dimethylbutane.

*Example VI*

Following the procedure of Example I, from 300 parts by weight of isobutane, 300 parts by weight of propane and 100 parts by weight of tert.-butyl hydroperoxide heated at a temperature of 320° F. and a pressure of 1100 p. s. i. g. for 12 hours were produced 0.4 gram of highly branched paraffins.

*Example VII*

Following the procedure of Example I, from 300 parts by weight of isobutane, 300 parts by weight of propane and 100 parts by weight of benzoyl peroxide heated at a temperature of 212° F. and a pressure of 500 p. s. i. g. for 48 hours were produced about 0.4 gram of C<sub>6</sub> to C<sub>7</sub> branched paraffin hydrocarbons.

*Example VIII*

Following the procedure of Example I, from 180 parts by weight of isobutane, 180 parts by weight of propane and 100 parts by weight of lauroyl peroxide heated at a temperature of 212° F. and a pressure of 575 p. s. i. g. for 24 hours were produced only traces of C<sub>6</sub>+ branched hydrocarbons.

*Example IX*

Following the procedure of Example I, omitting the inclusion of any di-(tert.-butyl) peroxide, only traces of a liquid product were obtained.

*Example X*

Following the procedure of Example I, omitting both isobutane and propane, only traces of a liquid product were observed.

I claim:

1. A process for preparing highly branched aliphatic hydrocarbons which comprises heating a lower paraffin in the presence of at least one peroxide selected from the group consisting of dialkyl peroxides, alkyl hydroperoxides and acyl peroxides, said heating being at a temperature between about 150 and 400° F., sufficient to effect decomposition of the peroxide.

2. A process for preparing highly branched aliphatic hydrocarbons which comprises heating a mixture of lower paraffins in the presence of a dialkyl peroxide, said heating being at a temperature between about 150 and 400° F., sufficient to effect decomposition of the peroxide.

3. A process for preparing highly branched aliphatic hydrocarbons which comprises heating a lower paraffin and propane in the presence of a lower dialkyl peroxide, said heating being at a temperature between about 150 and 400° F., sufficient to effect decomposition of the peroxide.

4. A process for preparing highly branched aliphatic hydrocarbons which comprises heating at least one lower paraffin in the presence of from 0.02 to 0.5 mole of a peroxide per mole of lower paraffin, said heating being at a temperature between about 150 and 400° F., sufficient to effect decomposition of the peroxide.

5. A process for preparing highly branched aliphatic hydrocarbons which comprises heating a mixture of lower paraffins in the presence of from 0.02 to 0.5 mole of at least one dialkyl peroxide per mole of said paraffin mixture, said heating being at a temperature between about 150 and 400° F., sufficient to effect decomposition of the peroxide.

6. A process for preparing highly branched aliphatic hydrocarbons which comprises heating a mixture of propane and isobutane in the presence of from 0.02 to 0.5 mole of di-(tert.-butyl) peroxide per mole of said mixture, said heating being at a temperature between about 150 and 400° F., sufficient to effect decomposition of the peroxide.

References Cited in the file of this patent

UNITED STATES PATENTS

|           |                      |                |
|-----------|----------------------|----------------|
| 2,270,669 | De Simo et al. ----- | Jan. 20, 1942  |
| 2,306,253 | McMillan -----       | Dec. 22, 1942  |
| 2,385,344 | Burk -----           | Sept. 25, 1945 |
| 2,530,874 | Gwynn et al. -----   | Nov. 21, 1950  |